

3,726,728

**BINDERLESS CAST PHOTOFASL COMPOSITIONS**  
 Howard W. Kruse, Ridgecrest, and Bertram A. Breslow,  
 China Lake, Calif., and Raymond W. Szypulski, Berwin  
 Heights, Md., assignors to the United States of America  
 as represented by the Secretary of the Navy  
 No Drawing. Filed Apr. 20, 1970, Ser. No. 30,328  
 Int. Cl. C06b 11/00

U.S. CL. 149—17

6 Claims

**ABSTRACT OF THE DISCLOSURE**

A binderless cast photoflash composition consisting of about 40% by weight metal powder dispersed in about 60% by weight molten inorganic oxidizer. This composition is less sensitive to impact, friction, and static electricity than flash powders consisting of finely divided loose-powder metal and oxidizer mixtures.

**GOVERNMENT INTEREST**

The invention described herein may be manufactured and used by or for the Government of the United States of America for governmental purposes without the payment of any royalties thereon or therefor.

**BACKGROUND OF THE INVENTION**

This invention relates to a binderless cast photoflash composition consisting of a low-melting inorganic oxidizer and a powdered metal.

Photoflash cartridges and bombs used in night aerial reconnaissance photography contain a loose-powder pyrotechnic charge which is a metal and an oxidizer in a finely divided condition. These photoflash powders are hazardous in any quantity in that they are highly sensitive to impact, friction, and static electricity. The processing and the manufacture of cartridges or bombs is one of the most hazardous in pyrotechnics. The problems encountered in the creation of a fire ball from a flash charge, its development, duration, size, shape, useful light output, etc., depend on many factors and are even more complex than the problems of ordinary pyrotechnic flames. The present invention provides a photoflash composition which is comparatively safe to manufacture and handle.

**DESCRIPTION OF THE INVENTION**

In accordance with the present invention a photoflash composition was prepared by adding metal powder to melted oxidizer in suitable heated mixing equipment and then pouring the mixture into a charge case. Alternatively, a mixture of coarse oxidizer and metal powder can be heated until the oxidizer melts, the mixture stirred, and then poured into the charge case. The mixture can be loaded into the casing, then heated until the oxidizer melts and the entire mass compacted by vibration. A typical photoflash composition in accordance with this invention contains about 40% by weight metal powder and about 60% molten oxidizer. The preferred metal is aluminum. The preferred oxidizer includes a mixture of salts selected from the group consisting of potassium perchlorate, lithium perchlorate, ammonium perchlorate, sodium perchlorate, and calcium perchlorate. The metal to oxidizer weight ratio ranges from 40:60 to 60:40.

The following examples will better illustrate this invention.

**Example I**

60% by weight of a prefused eutectic mixture comprising a blend of 68.6% lithium perchlorate and 31.4% sodium perchlorate was melted in an open crucible by heat-

ing to about 207° C. The melt was maintained at about 230–250° C. while 40% by weight powdered aluminum (20 $\mu$ ) was added while mixing with a spatula. The resultant slurry was cast into small test cartridges containing 120–130 grams. The cartridges were steel cases 1 $\frac{1}{4}$ " x 3 $\frac{3}{8}$ " having a 1/4" Teflon mandrel positioned in the center. The slurry was cast around the mandrel and permitted to cool at room temperature thereby forming a solid. The mandrel was removed and the well formed was later filled with a high explosive to trigger the photoflash composition. Two explosives were used; one, an extruded explosive containing 85% HMX with 15% Viton-Teflon binder, and the other was tetryl in the form of pressed pellets.

The average peak candlepower of 32 cartridges containing this cast binderless composition which were made and tested over a period of one year was  $33.4 \times 10^6$ .

**Example II**

50% by weight of the same eutectic mixture, lithium/sodium perchlorate and 50% by weight powdered aluminum were prepared as described in Example I. Six cartridges containing this composition were tested and averaged a peak candlepower of  $50.2 \times 10^6$ . The 50:50 metal to oxidizer ratio is much thicker than the 40:60 ratio described in Example I, but still can be cast by pouring and the peak candlepower is increased.

**Example III**

Example I was repeated several times substituting for the LiCl<sub>4</sub>—NaClO<sub>4</sub> eutectic mixture the following blends of perchlorates and maintaining the molten mixture 20–30° C. above the indicated melting temperature: 57% LiClO<sub>4</sub>—21.6% NaClO<sub>4</sub>—21.4% Ca(ClO<sub>4</sub>)<sub>2</sub> (202° C.); 66% LiClO<sub>4</sub>—34% NH<sub>4</sub>ClO<sub>4</sub> (182° C.); 70.8% LiClO<sub>4</sub>—29.2% KClO<sub>4</sub> (207° C.). These compositions were cast and tested as in Example I. The light output of each compared favorably with the lithium/sodium perchlorate-aluminum photoflash composition set out hereinabove.

M123-size flash charges containing 40%, 45%, 50% and 55% aluminum powder (20 micron) and the lithium perchlorate-sodium perchlorate eutectic mixture with a one-inch tetryl burster were prepared and tested. Average peak candlepower of these devices was approximately  $300 \times 10^6$  CP (range 240–340  $\times 10^6$  CP) and there was no appreciable change in peak with increasing metal content. Increase in metal content resulted in a higher integral light output, however. This increase in integral (or total) light was small over the first 10 milliseconds, but became greater over 40 milliseconds.

The perchlorate oxidizers used herein are comparatively safe to handle and give excellent light output. The casing may be of the usual steel, glass tape, plastic or other suitable material so long as the atmospheric moisture is kept away from the cast composition and the casing material is compatible with the composition.

What is claimed is:

1. A photoflash composition having a continuous solid phase and a dispersed solid phase; said continuous phase comprising from 40 to 60% by weight of a mixture of oxidizers selected from the group consisting of potassium perchlorate, lithium perchlorate, sodium perchlorate, ammonium perchlorate and calcium perchlorate; and said dispersed phase comprising from 40 to 60% by weight finely divided particulate aluminum; said composition producing a flash having a peak candlepower in the range of from about  $33.4 \times 10^6$  to about  $340 \times 10^6$  when activated.

2. The composition according to claim 1 in which the continuous phase approximates a eutectic mixture.

3. The composition according to claim 1 in which the continuous phase is a eutectic mixture consisting essentially of lithium perchlorate and sodium perchlorate.

4. A composition according to claim 1 in which the continuous phase is a eutectic mixture consisting essentially of lithium perchlorate and ammonium perchlorate.

5. A composition according to claim 1 in which the continuous phase is a eutectic mixture consisting essentially of lithium perchlorate and potassium perchlorate.

6. A composition according to claim 1 in which the ratio of oxidizer to aluminum is about equal.

## References Cited

## UNITED STATES PATENTS

|           |         |                |          |
|-----------|---------|----------------|----------|
| 3,106,497 | 10/1963 | Weil           | 149—17   |
| 3,293,187 | 12/1966 | Markowitz      | 149—40 X |
| 3,331,203 | 7/1967  | Kaufman et al. | 149—17 X |
| 3,522,334 | 7/1970  | Hunter et al.  | 149—17 X |

CARL D. QUARFORTH, Primary Examiner

10 P. A. NELSON, Assistant Examiner

U.S. CL. X.R.

149—40, 76, 77, 113; 431—93